

## UNITED STATES PATENT OFFICE

2,345,096

## CATALYTIC CONVERSION OF HYDRO-CARBONS

Robert E. Burk and Everett C. Hughes, Cleveland Heights, Ohio, assignors to The Standard Oil Company, Cleveland, Ohio, a corporation of Ohio

No Drawing. Application April 29, 1941,  
Serial No. 390,960

13 Claims. (Cl. 260—668)

This invention relates to conversion of hydrocarbons, and it is among the objects of the invention to catalytically raise the aromatic content of hydrocarbons or convert non-benzenoid hydrocarbons to aromatics, and inhibit deposition of coke on the catalyst and facilitate the heating. Other objects and advantages will appear as the description proceeds.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

The hydrocarbons to be treated may be of any desired non-benzenoid character, as aliphatic hydrocarbons or paraffins and olefins and naphthenic hydrocarbons or their mixtures, naphthas, distillates, etc. The catalyst or contact material is of peculiar composition, being a gel type coprecipitated combination of oxides of copper, aluminum and chromium, the copper oxide being 1-10 mol per cent, the aluminum oxide 81-60 mol per cent, and the chromium oxide 18-30 mol per cent. The operating temperature for the catalyst is 750° F. and upward. With the hydrocarbon feed there may be supplied a hydrocarbon gas of four carbon atoms or in some cases less. Such butane gas may be supplied at the rate of 1-10 mols per mol of naphtha or the like fed. Preferably, a supply of hydrogen is also provided. This may be in amount 0.1-10 mols per mol of naphtha or the like. Off-gas from the process containing a butane hydrocarbon and hydrogen may conveniently be employed, being returned to the catalyst zone. Where the arrangement of the catalyst involves a series of trays or beds through which the hydrocarbon feed is passed, it is advantageous to supply the gas additions in successive portions to at least a part of the trays of catalyst, as many as desired. With this kind of catalyst and a supply of hydrogen, incipient coke-forming material is hydrogenated, with exothermic heat generation providing heat in situ also at the catalyst bed. Flow rates of naphtha may be 0.1-10 liquid volumes per volume of catalyst per hour. At the higher temperature ranges correspondingly shorter contact times may be employed. In operating with supply of hydrogen, the temperature may be slightly higher than those used ordinarily in aromatization. Temperatures of 750-1200° F. are applicable. The

operating pressure may vary, depending upon other conditions. Thus, where introducing hydrogen as the only additional gas fed into the catalyst zone, the pressure may be as high as 400 lbs. per square inch; where butane is employed the pressure may be up to 800 lbs. for instance; and commonly the pressure may be 40-400 lbs.

The products from the catalytic zone, after separating the gases which may be returned in such amount as desired, may be extracted with a selective solvent or mixture, as for instance liquid sulphur dioxide or a high boiling amine or a hydroxy compound etc., and the undissolved or non-benzenoid portion may be returned to the catalytic zone. The catalyst may be regenerated in situ by shutting off the feed and applying to it while the temperature is at 750-1200° F., an oxygen-containing gas such as air or oxygen which may be diluted with a suitable diluent, for instance nitrogen.

As an example: A naphtha from Illinois petroleum is passed in contact with a co-precipitated gel type oxide catalyst consisting of 2 mol per cent of copper oxide, 78 mol per cent of aluminum oxide, and 20 mol per cent of chromium oxide, at a temperature of 980° F., and pressure 100 pounds per square inch, and a flow rate of 1 mol of naphtha (liquid) per volume of catalyst per hour, and hydrogen supplied at the rate of 3 mols of hydrogen per mol of naphtha. A yield of 73.3 weight per cent of gasoline is obtained, having a Katt-winkel test of 54 and A. S. T. M. octane number (without butane) of 79.7. Operating with the same conditions as foregoing, and adding also 1.17 mols of butane gas per mol of naphtha, an 84.3 per cent yield of gasoline is obtained having an A. S. T. M. number of 75.

This application is a continuation, in part and as to common subject matter, of our application Serial No. 263,198, filed March 21, 1939.

Other modes of applying the principle of the invention may be employed, change being made as regards the details described, provided the features stated in any of the following claims, or the equivalent of such, be employed.

We therefore particularly point out and distinctly claim as our invention:

1. A process of raising the aromatic content of hydrocarbons, which comprises maintaining at about 750-1200° F. a gel type catalyst containing 1-10 mol per cent of copper oxide and 81-60 mol per cent of aluminum oxide coprecipitated with 18-30 mol per cent of chromium oxide, and contacting a vaporized naphtha with such catalyst while supplying a butane hydrocarbon and hydro-

gen in mol ratio of 1-10 and 0.1-10 respectively to 1 of the naphtha, and maintaining superatmospheric pressure.

2. A process of raising the aromatic content of hydrocarbons, which comprises maintaining at about 750-1200° F. a series of bodies of a gel type catalyst containing 1-10 mol per cent of copper oxide and 81-60 mol per cent of aluminum oxide coprecipitated with 18-30 mol per cent of chromium oxide, and passing through the series a vaporized naphtha while supplying to at least a part of the series of catalyst bodies a butane hydrocarbon and hydrogen in mol ratio of 1-10 and 0.1-10 respectively to 1 of the naphtha, and maintaining superatmospheric pressure.

3. A process of raising the aromatic content of hydrocarbons, which comprises maintaining at about 750-1200° F. a gel type catalyst containing 1-10 mol per cent of copper oxide and 81-60 mol per cent of aluminum oxide coprecipitated with 18-30 mol per cent of chromium oxide, and contacting a vaporized naphtha with the catalyst while supplying a butane gas and hydrogen in mol ratio of 1-10 and 0.1-10 respectively to 1 of the naphtha, and returning off-gas to the catalyst zone.

4. A process of raising the aromatic content of hydrocarbons, which comprises maintaining at about 750-1200° F. a gel type catalyst containing 1-10 mol per cent of copper oxide and 81-60 mol per cent of aluminum oxide coprecipitated with 18-30 mol per cent of chromium oxide, and contacting a vaporized naphtha with the catalyst while supplying a butane gas in mol ratio of 1-10 to 1 of the naphtha, and returning non-benzenoid hydrocarbons from the product to the catalyst.

5. A process of raising the aromatic content of hydrocarbons, which comprises maintaining at about 750-1200° F. a series of bodies of a gel type catalyst containing 1-10 mol per cent of copper oxide and 81-60 mol per cent of aluminum oxide coprecipitated with 18-30 mol per cent of chromium oxide, and passing through the series a vaporized naphtha while supplying to at least a part of the series of catalyst bodies hydrogen in mol ratio of 0.1-10 to 1 of the naphtha, and maintaining superatmospheric pressure.

6. A process of raising the aromatic content of hydrocarbons, which comprises maintaining at about 750-1200° F. a gel type catalyst containing 1-10 mol per cent of copper oxide and 81-60 mol per cent of aluminum oxide coprecipitated with 18-30 mol per cent of chromium oxide, and passing in contact with such catalyst an aromatizable non-benzenoid hydrocarbon, while supplying a butane gas and hydrogen in mol ratio of 1-10 and 0.1-10 respectively to 1 of the hydrocarbon, and maintaining superatmospheric pressure.

7. A process of raising the aromatic content of hydrocarbons, which comprises maintaining at about 750-1200° F. a series of bodies of a gel type catalyst containing 1-10 mol per cent of copper oxide and 80-60 mol per cent of aluminum oxide coprecipitated with 18-30 mol per cent of chromium oxide, and passing through the series an aromatizable non-benzenoid hydrocarbon, while supplying to at least a part of the series of catalyst bodies a butane hydrocarbon and hydrogen in mol ratio of 1-10 and 0.1-10 respectively to 1 of

the hydrocarbon, and maintaining superatmospheric pressure.

8. A process of raising the aromatic content of hydrocarbons, which comprises maintaining at about 750-1200° F. a gel type catalyst containing 1-10 mol per cent of copper oxide and 80-60 mol per cent of aluminum oxide coprecipitated with 18-30 mol per cent of chromium oxide, and contacting an aromatizable non-benzenoid hydrocarbon with the catalyst, while supplying a butane hydrocarbon and hydrogen in mol ratio of 1-10 and 0.1-10 respectively to 1 of the hydrocarbon.

9. A process of raising the aromatic content of hydrocarbons, which comprises maintaining at elevated temperature a gel type catalyst containing 1-10 mol per cent of copper oxide and 81-60 mol per cent of aluminum oxide coprecipitated with 18-30 mol per cent of chromium oxide, and passing an aromatizable non-benzenoid hydrocarbon in contact with such catalyst, while supplying a butane hydrocarbon and hydrogen in mol ratio of 1-10 and 0.1-10 respectively to 1 of the hydrocarbon, and returning off-gas to the catalyst zone.

10. A process of raising the aromatic content of hydrocarbons, which comprises maintaining at elevated temperature a gel type catalyst containing 1-10 mol per cent of copper oxide and 81-60 mol per cent of aluminum oxide coprecipitated with 18-30 mol per cent of chromium oxide, and passing an aromatizable non-benzenoid hydrocarbon in contact with such catalyst, while supplying a butane gas and hydrogen in mol ratio of 1-10 and 0.1-10 respectively to 1 of the hydrocarbon, and returning non-benzenoid hydrocarbons from the product to the catalyst.

11. A process of raising the aromatic content of hydrocarbons, which comprises maintaining at elevated temperature a gel type catalyst containing 1-10 mol per cent of copper oxide and 81-60 mol per cent of aluminum oxide coprecipitated with 18-30 mol per cent of chromium oxide, and passing an aromatizable non-benzenoid hydrocarbon in contact with such catalyst, while supplying hydrogen in mol ratio of 0.1-10 to 1 of the hydrocarbon, and maintaining superatmospheric pressure.

12. A process of converting hydrocarbons to aromatics, which comprises subjecting non-benzenoid hydrocarbons in the presence of a portion of off-gas returned from the process to the action, at 750-1200° F., of a contact mass characterized by 1-10 mol per cent of copper oxide with 60-81 mol per cent of gel type aluminum oxide which is coprecipitated with 18-30 mol per cent of chromium oxide.

13. A process of converting hydrocarbons to aromatics, which comprises subjecting a non-benzenoid hydrocarbon containing naphtha in the presence of a portion of off-gas returned from the process to the action, at 750-1200° F., of a contact mass characterized by 1-10 mol per cent of copper oxide with 60-81 mol per cent of gel type aluminum oxide which is coprecipitated with 18-30 mol per cent of chromium oxide.

ROBERT E. BURK  
EVERETT C. HUGHES.